# EUROPEAN PATENT SPECIFICATION

(11) **EP 3 690 086 B1**
(45) Date of publication and mention of the grant of the patent: **25.05.2022**
(21) Application number: 18900577.0
(22) Date of filing: 21.12.2018
(51) Int. Cl.: D01D 5/088, D01D 5/098

(54) **MELT SPINNING APPARATUS AND NON-WOVEN FABRIC PRODUCTION METHOD**
SCHMELZSPINNVORRICHTUNG UND VERFAHREN ZUR HERSTELLUNG VON VLIESSTOFF
APPAREIL DE FILAGE PAR FUSION ET PROCÉDÉ DE PRODUCTION D'UN TISSU NON-TISSÉ

(43) Date of publication of application: 05.08.2020
(73) Proprietor: Mitsui Chemicals, Inc., Minato-ku Tokyo 105-7122 (JP)
(72) Inventor: ODOI, Masaaki, Sodegaura-shi Chiba 299-0265 (JP); KAWADA, Atsushi, Sodegaura-shi Chiba 299-0265 (JP); YOKOYAMA, Tetsuya, Sodegaura-shi Chiba 299-0265 (JP)
(74) Representative: Hoffmann Eitle
(86) International application number: PCT/JP2018/047370
(87) International publication number: WO 2020/129256

(56) References cited:
- EP-A1- 1 396 568
- JP-A- S63 275 767
- JP-A- 2007 046 224
- JP-U- H0 322 070
- JP-U- S4 998 506
- JP-U- S50 119 708
- JP-Y1- S4 636 421
- US-A- 3 070 839
- US-A- 3 999 910
- US-A- 5 173 310
- US-A1- 2003 178 742

## Description

### Technical Field

The present disclosure relates to a melt spinning apparatus and to a method of manufacturing a non-woven fabric.

### Background Art

Examples of methods of manufacturing spunbonded non-woven fabrics include a method in which spun filaments are cooled by cooling air introduced into a cooling chamber, drawn through nozzles using cooling air as drawing air on an as-is basis, and scattered on a mesh belt.

In a step of manufacturing a spunbonded non-woven fabric, cooling air is sprayed on a large number of continuous filaments melt-spun from spinning nozzles, thereby cooling the filaments. A sufficient volume of cooling air is needed in the case of increasing the amount of discharged filaments in order to enhance productivity in such a case. A small volume of cooling air results in insufficient cooling of the filaments, thereby causing a resin block (shot) to be prone to be generated on a web. In contrast, a large volume of cooling air causes yarn breakage to be prone to occur due to supercooling.

Thus, a method and apparatus of manufacturing a non-woven fabric, in which yarn breakage does not occur even in the case of increasing the volume of cooling air, a fiber diameter can be reduced without deteriorating productivity, and a non-woven fabric can be stably manufactured, are proposed (see, for example, Patent Document 1). Specifically, Patent Document 1 proposes the method of manufacturing a non-woven fabric, in which cooling air introduced into a cooling chamber is divided into at least two stages in a vertical direction, and the air velocity of cooling air in a bottom stage is allowed to be higher than the air velocity of cooling air in a top stage.

### Citation List

### Patent Document

Patent Document 1: Japanese Patent Application Laid-Open (JP-A) No. 2002-317372

### SUMMARY OF INVENTION

### Technical Problem

However, the method and apparatus of manufacturing a non-woven fabric, proposed in Patent Document 1, have a problem that the uniformity (texture) of the mass distribution of an overall non-woven fabric is prone to be deteriorated, whereby so-called yarn fluctuation is prone to occur.

The present invention was made under such circumstances with an object of providing a melt spinning apparatus in which yarn breakage and yarn fluctuation can be suppressed, and a method of manufacturing a non-woven fabric using the apparatus.

### Solution to Problem

Specific means for addressing the above problem include the following aspects.
<1> A melt spinning apparatus comprising:
   a spinning unit comprising a plurality of spinning nozzles that spin filaments;
   a cooling unit that cools the filaments spun from the spinning nozzles; and
   a cooling air supply unit that faces the cooling unit and supplies cooling air to the cooling unit through an air-permeable partition,
   wherein the cooling air supply unit comprises a first cooling air supply unit at a vertically upper side and a second cooling air supply unit at a vertically lower side, divided into two stages in a vertical direction through a partition, there is a gap between an end of the partition facing the air-permeable partition and a face of a side of the air-permeable partition facing the partition, and a distance of the gap (d) is 55 mm or less.
   Further, the distance of the gap is 5 mm or more.
<2> The melt spinning apparatus according to <1>, wherein a ratio of a distance (B) from a nozzle face, on which the spinning nozzles of the spinning unit are disposed, to the partition, with respect to the distance of the gap (d), is from 5 to 50.
<3> The melt spinning apparatus according to any one of <1> to <2>, wherein a ratio of a height (h₂) of the second cooling air supply unit, to a height (h₁) of the first cooling air supply unit, is from 0.5 to 1.5.
<4> The melt spinning apparatus according to any one of <1> to <3>, wherein a thickness of the air-permeable partition is from 10 mm to 50 mm.
<5> The melt spinning apparatus according to any one of <1> to <4>, wherein a ratio of a thickness of the air-permeable partition to the distance of the gap (d) is from 0.5 to 5.0.
<6> The melt spinning apparatus according to any one of <1> to <5>, wherein the air-permeable partition has a honeycomb shape.
<7> The melt spinning apparatus according to any one of <1> to <6>, wherein the cooling air supply unit comprises a flow regulating plate that regulates the cooling air supplied to the cooling unit, upstream of the air-permeable partition, in a direction of cooling air supply.
<8> The melt spinning apparatus according to any one of <1> to <7>, further comprising a first controller that performs control so that a temperature of cooling air supplied to the first cooling air supply unit is from 10°C to 40°C, and a temperature of cooling air supplied to the second cooling air supply unit is higher than the temperature of the cooling air supplied to the first cooling air supply unit by 10°C or more and is from 30°C to 70°C.
<9> The melt spinning apparatus according to any one of <1> to <8>, further comprising a second controller that performs control so that a ratio (V₁/V₂) of an average air velocity (V₁) of cooling air supplied to the first cooling air supply unit, with respect to an average air velocity (V₂) of cooling air supplied to the second cooling air supply unit, is from more than 0 to 0.7.
<10> The melt spinning apparatus according to any one of <1> to <9>, further comprising a drawing unit that draws the filaments cooled in the cooling unit,
   wherein a ratio of a distance (B) from a nozzle face, on which the spinning nozzles of the spinning unit are disposed, to the partition, with respect to a distance (C) from the nozzle face, on which the spinning nozzles of the spinning unit are disposed, to an inlet of the drawing unit (= distance B/distance C), is from 0.2 to 0.8.
<11> The melt spinning apparatus according to any one of <1> to <10>, further comprising a collecting unit that collects cooled and drawn filaments to form a non-woven web, wherein the melt spinning apparatus is used for manufacturing a spunbonded non-woven fabric.
<12> A method of manufacturing a non-woven fabric, comprising manufacturing a non-woven fabric from filaments spun from the plurality of spinning nozzles using the melt spinning apparatus according to any one of <1> to <11>.
<13> The method of manufacturing a non-woven fabric according to <12>, wherein a temperature of cooling air supplied to the first cooling air supply unit is from 10°C to 40°C, and a temperature of cooling air supplied to the second cooling air supply unit is higher than the temperature of the cooling air supplied to the first cooling air supply unit by 10°C or more and is from 30°C to 70°C.
<14> The method of manufacturing a non-woven fabric according to <12> or <13>, wherein a ratio (V₁/V₂) of an average air velocity (V₁) of cooling air supplied to the first cooling air supply unit, with respect to an average air velocity (V₂) of cooling air supplied to the second cooling air supply unit, is from more than 0 to 0.7.
<15> The method of manufacturing a non-woven fabric according to any one of <12> to <14>, wherein the filaments comprise a propylene-based polymer.

### Advantageous Effects of Invention

The present disclosure can provide a melt spinning apparatus in which yarn breakage and yarn fluctuation can be suppressed, and a method of manufacturing a non-woven fabric using the apparatus.

### BRIEF DESCRIPTION OF DRAWINGS

Fig. 1 is a schematic configuration view illustrating a partial cross section of a melt spinning apparatus of the present disclosure.
Fig. 2 is a graph indicating a relationship between the height of a cooling air supply unit and the air velocity (outlet value) of cooling air in Examples 1 to 3.
FIG. 3 is a graph indicating a relationship between the height of a cooling air supply unit and the air velocity (outlet value) of cooling air in Examples 1 to 3 and Comparative Examples 1 to 6.

### DESCRIPTION OF EMBODIMENTS

Specific embodiments of the invention will be described in detail below. However, the invention is not limited to the embodiments described below, and can be modified and carried out within the scope of an object of the invention, if appropriate.

In the present disclosure, any numerical value range indicated by the term "to" represents any range including the numerical values described before and after the term "to" as the lower limit value and the upper limit value, respectively.

In a numerical range expressed in a stepwise manner in the present disclosure, the upper or lower limit value expressed in one numerical range may be replaced by the upper or lower limit value in another numerical range expressed in a stepwise manner. In a numerical range expressed in the present disclosure, the upper or lower limit value of the numerical range may be replaced by values described in Examples.

In the present disclosure, in a case in which an embodiment is explained with reference to a drawing, the configuration of the embodiment is not limited to a configuration illustrated in the drawing. The sizes of members in each drawing are conceptual, and the relative relationships between the sizes of the members are not limited thereto.

### [Melt Spinning Apparatus]

A melt spinning apparatus of the present disclosure includes a spinning unit including plural spinning nozzles that spin filaments, a cooling unit that cools the filaments spun from the spinning nozzles, and a cooling air supply unit that faces the cooling unit and supplies cooling air to the cooling unit through an air-permeable partition, wherein the cooling air supply unit includes a first cooling air supply unit at a vertically upper side and a second cooling air supply unit at a vertically lower side, divided into two stages in a vertical direction through a partition, there is a gap between an end, facing the air-permeable partition, of the partition and a face of a side, facing the partition, in the air-permeable partition, and the distance of the gap d is 55 mm or less and 5 mm or more.

The melt spinning apparatus of the present disclosure includes the cooling air supply unit including the first cooling air supply unit at the vertically upper side and the second cooling air supply unit at the vertically lower side, divided into the two stages in the vertical direction through the partition, and includes the gap between the end, facing the air-permeable partition, of the partition and the face of the side, facing the partition, in the air-permeable partition, wherein the distance of the gap d is 55 mm or less and 5 mm or more. It is presumed that as a result, a difference between the air velocities of cooling airs in the boundary of the first cooling air supply unit at the vertically upper side and the second cooling air supply unit at the vertically lower side, in the cooling unit, can be decreased, the cooling airs with the small air velocity difference in the vicinity of the boundary are supplied to the filaments, and therefore, turbulence caused by mixing the cooling airs having different air velocities is suppressed, whereby yarn breakage and yarn fluctuation can be suppressed.

The configuration of the melt spinning apparatus of the present disclosure will be described below with reference to Fig. 1. As illustrated in Fig. 1, the melt spinning apparatus 100 includes a spinning unit 1, a cooling chamber (cooling unit) 3, a cooling air supply unit 4, an air-permeable partition 8, and a drawing unit 9. The cooling air supply unit 4 is divided into two stages through a partition 7, and includes a first cooling air supply unit 5 at a vertically upper side and a second cooling air supply unit 6 at a vertically lower side. There is a gap between an end, facing the air-permeable partition 8, of the partition 7 and a face of a side, facing the partition 7, in the air-permeable partition 8.

The melt spinning apparatus 100 is an apparatus that discharges a resin composition supplied to the spinning unit 1, from plural spinning nozzles into the cooling chamber 3, and cools and draws the discharged filaments. The melt spinning apparatus 100 may be an apparatus used for manufacturing a spunbonded non-woven fabric, and may include, for example, a collecting unit that forms a non-woven web on which the cooled and drawn filaments are deposited, and an entanglement unit that subjects the non-woven web to heating and pressurization treatment.

The melt spinning apparatus 100 includes the spinning unit 1 including the plural spinning nozzles through which filaments are spun. For example, a resin composition melt-kneaded with an extruder is supplied to the spinning unit 1, and the resin composition supplied to the spinning unit 1 is discharged as filaments from the plural spinning nozzles disposed on a nozzle face 2 into the cooling chamber 3.

The resin composition may include a resin used for manufacturing a non-woven fabric. Examples of the resin used for manufacturing a non-woven fabric include a polyester resin, a polyurethane resin, a polyamide resin, and a polyolefin resin. Especially, a polyolefin resin is preferred, and a propylene-based polymer is more preferred, in view of excellent productivity.

The propylene-based polymer may be a polymer including propylene as a constitutional unit, may be a propylene homopolymer, may be a propylene random copolymer, or may be a mixture thereof.

The propylene random copolymer is preferably a random copolymer in which the content of propylene with respect to all constitutional units is 50% by mol or more. The propylene random copolymer is preferably a propylene α-olefin random copolymer.

In the propylene random copolymer, the content of propylene with respect to all the constitutional units is preferably from 70% by mol to 99.5% by mol, more preferably from 80% by mol to 98% by mol, and still more preferably from 90% by mol to 96% by mol.

The α-olefin is preferably an α-olefin having two or more carbon atoms, excluding propylene, more preferably an α-olefin having 2 or from 4 to 8 carbon atoms, and still more preferably ethylene which is an α-olefin having 2 carbon atoms.

Specific examples of the α-olefin include ethylene, 1-butene, 1-pentene, 1-hexene, 1-octene, and 4-methyl-1-pentene.

Such α-olefins may be used singly, or in combination two or more kinds thereof.

The resin composition may include another component as well as the resin used for manufacturing a non-woven fabric. Examples of the other component include another polymer, an organic peroxide, a surfactant, a coloring agent, an antioxidant based on phosphorus, phenol, or the like, a weathering stabilizer based on benzotriazole or the like, a light stabilizer based on a hindered amine or the like, an anti-blocking agent, a dispersant such as calcium stearate, a lubricant, a nucleating agent, a pigment, a softening agent, a hydrophilization agent, a water repellent, an aid, a water repellent, a filler, an antibacterial agent, a pesticide, an insect repellent, an agent, a natural oil, and a synthetic oil.

The melt spinning apparatus 100 includes the cooling chamber 3 in which filaments spun from the spinning nozzles are cooled. Cooling air is supplied from the cooling air supply unit 4 into the cooling chamber 3 through the air-permeable partition 8, and the filaments are cooled by the supplied cooling air. An exhaust-nozzle for exhausting a vapor of low-molecular-weight polymer may be mounted between the nozzle face 2, which is an upper portion of the cooling chamber 3, and the cooling air supply unit 4.

The melt spinning apparatus 100 includes the cooling air supply unit 4 that faces the cooling chamber 3 and supplies cooling air to the cooling chamber 3 through the air-permeable partition 8. The cooling air supply unit 4 includes the first cooling air supply unit 5 at the vertically upper side and the second cooling air supply unit 6 at the vertically lower side, divided into two stages in a vertical direction. As illustrated in Fig. 1, the first cooling air supply unit 5 and the second cooling air supply unit 6 supply cooling airs in the directions of arrows in Fig. 1.

As illustrated in Fig. 1, such cooling air supply units 4 supply cooling airs from two directions, facing each other, to the cooling chamber 3 through such air-permeable partitions 8, respectively.

The cooling air supply unit 4 may include a flow regulating plate that regulates cooling air supplied to the cooling chamber 3, upstream of the air-permeable partition 8 in the direction of cooling air supply. As a result, the direction of cooling air supplied to the cooling chamber 3 is regulated, and yarn breakage and yarn fluctuation can be more preferably suppressed.

It is preferable that (L × h)/d satisfies 0.056 or more assuming that the width of the cooling air supply unit 4 is L (m), the height of the cooling air supply unit 4 is h (m), and the distance of the gap is d (mm). In such a case, the height h of the cooling air supply unit 4 corresponds to h₁ + h₂ + the thickness of the partition 7 in Fig. 1, and the width of the cooling air supply unit 4 is the length of the inner side of the cooling air supply unit 4, excluding an outer wall, in the direction orthogonal to the direction of cooling air supply and the height of the cooling air supply unit 4 in Fig. 1.

The width L of the cooling air supply unit 4 and the height h of the cooling air supply unit 4 means the width and height of the cooling air outlet of the cooling air supply unit 4. Accordingly, (L × h) means the area of a face, through which cooling air passes, of the cooling air outlet of the cooling air supply unit 4, and (L × h)/d means the ratio of the area to the distance d of the gap.

(L × h)/d may be from 0.056 to 0.614, or may be from 0.112 to 0.448. Yarn breakage can be more preferably suppressed in a case in which (L × h)/d is 0.056 or more, and yarn fluctuation can be more preferably suppressed in a case in which (L × h)/d is 0.614 or less.

The distance d of the gap may be 50 mm or less, may be 45 mm or less, and may be 40 mm or less, in view of more preferably suppressing yarn breakage.

The numerical value of the distance d of the gap is not particularly limited as long as the gap is present. The distance d may be 5 mm or more, and may be 10 mm or more, in view of more preferably suppressing yarn fluctuation.

The width L of the cooling air supply unit 4 is not particularly limited. The width L may be from 3 m to 7 m, and may be from 4 m to 6 m. The height of the cooling air supply unit 4 is not particularly limited. The height may be from 0.4 m to 1.0 m, and may be from 0.6 m to 0.8 m.

The ratio of a distance from the nozzle face 2 to the partition 7 with respect to the the distance d of the gap (distance from the nozzle face to the partition/ distance of the gap) may be from 5 to 50.

The ratio of the height (h₂) of the second cooling air supply unit 6 to the height (h₁) of the first cooling air supply unit 5 may be from 0.5 to 1.5, and may be from 0.8 to 1.2.

The melt spinning apparatus 100 may further include a first controller that controls the temperature (first temperature) of cooling air supplied to the first cooling air supply unit 5 and the temperature (second temperature) of cooling air supplied to the second cooling air supply unit 6.

The first temperature refers to the temperature of cooling air in the inlet of the first cooling air supply unit 5, and the second temperature refers to the temperature of cooling air in the inlet of the second cooling air supply unit 6.

In view of more preferably suppressing yarn breakage, the first controller preferably performs control so that the second temperature is higher than the first temperature, and more preferably performs control so that the first temperature is from 10°C to 40°C, and the second temperature is higher than the first temperature by 10°C or more and is from 30°C to 70°C.

The melt spinning apparatus 100 may further include a second controller that controls the average air velocity (V₁) of cooling air supplied to the first cooling air supply unit 5 and the average air velocity (V₂) of cooling air supplied to the second cooling air supply unit 6. The second controller may be the same as or different from the first controller.

V₁ refers to the average air velocity of cooling air in the inlet of the first cooling air supply unit 5, and V₂ refers to the average air velocity of cooling air in the inlet of the second cooling air supply unit 6.

The second controller preferably controls the average air velocity of cooling air so that V₂ is more than V₁ in view of preferably suppressing yarn breakage.

In view of more preferably suppressing yarn breakage, the second controller preferably performs control so that the ratio of V₁ to V₂ (V₁/V₂) is from more than 0 to 0.7, more preferably performs control so that 0.01 ≤ V₁/V₂ ≤ 0.5 is achieved, and still more preferably performs control so that 0.05 ≤ V₁/V₂ ≤ 0.4 is achieved.

The melt spinning apparatus 100 includes the air-permeable partition 8 that separates the cooling air supply unit 4 and the cooling chamber 3 from each other. The air-permeable partition 8 has permeability, and therefore, cooling air supplied from the cooling air supply unit 4 is introduced into the cooling chamber 3 through the air-permeable partition 8.

The air-permeable partition 8 is not particularly limited as long as the air-permeable partition 8 is a partition having permeability. In view of the regulation of cooling air, the air-permeable partition 8 preferably has a lattice shape such as a quadrangular shape, or a honeycomb shape such as a hexagonal shape or an octagonal shape, and more preferably has a honeycomb shape.

In view of strength and the regulation of cooling air, the thickness of the air-permeable partition 8 is preferably from 10 mm to 50 mm, and more preferably from 20 mm to 40 mm.

The ratio of the thickness of the air-permeable partition to the distance of the gap (thickness of air-permeable partition/distanced) is preferably from 0.5 to 5.0, more preferably from 0.5 to 1.5, and still more preferably from 0.8 to 1.2.

The melt spinning apparatus 100 further includes the drawing unit 9 that draws filaments cooled in the cooling chamber 3. The drawing unit 9 is a thin bottleneck that is arranged at the vertically lower side of the cooling chamber 3, and that is throttled from both right and left sides. In the drawing unit 9, cooling air has an increased air velocity, becomes drawing air, and allows the cooled filaments to be drawn.

The ratio of the distance B from the nozzle face 2 to the partition 7 with respect to a distance C from the nozzle face 2 to the inlet of the drawing unit 9 (distance B/distance C) is preferably from 0.2 to 0.8, and more preferably from 0.2 to 0.6.

### [Method of Manufacturing Non-Woven Fabric]

A method of manufacturing a non-woven fabric of the present disclosure is a method of manufacturing a non-woven fabric from filaments spun from plural spinning nozzles using the melt spinning apparatus of the present disclosure. Anon-woven fabric of which the yarn breakage and yarn fluctuation are suppressed can be obtained by the method.

The method of manufacturing a non-woven fabric of the present disclosure may include, for example, a step of discharging a resin composition, supplied to a spinning unit, from plural spinning nozzles into a cooling unit, a step of cooling discharged filaments, a step of drawing the cooled filaments, and a step of collecting the drawn filaments to form a non-woven web. The method of producing a non-woven fabric of the present disclosure may further include a step of subjecting the non-woven web to heating and pressurization treatment.

In view of more preferably suppressing yarn breakage, it is preferable that the temperature of cooling air supplied to a first cooling air supply unit is from 10°C to 40°C, and the temperature of cooling air supplied to a second cooling air supply unit is higher than the temperature of cooling air supplied to the first cooling air supply unit by 10°C or more and is from 30°C to 70°C.

In view of preferably suppressing yarn breakage, the average air velocity (V₂) of cooling air supplied to the second cooling air supply unit is preferably more than the average air velocity (V₁) of cooling air supplied to the first cooling air supply unit. In view of more preferably suppressing yarn breakage, the ratio of V₁ to V₂ (V₁/V₂) is preferably from more than 0 to 0.7, more preferably 0.01 ≤ V₁/V₂ ≤ 0.5, and still more preferably 0.05 ≤ V₁/V₂ ≤ 0.4.

The average air velocity (V₁') of cooling air supplied from the first cooling air supply unit to the cooling unit and the average air velocity (V₂') of cooling air supplied from the second cooling air supply unit to the cooling unit may be adjusted by controlling V₁ and V₂. For example, the ratio of V₁' to V₂' (V₁'/V₂') may be adjusted to be from more than 0 to 0.7, may be adjusted to be 0.01 ≤ V₁'/V₂' ≤ 0.5, and may be adjusted to be 0.1 ≤ V₁'/V₂' ≤ 0.5, by controlling V₁ and V₂.

### Examples

The invention will be more specifically described below with reference to Examples. However, the invention is not limited to the following Examples.

### [Examples 1 to 3 and Comparative Examples 1 to 6]

A non-woven fabric was manufactured using a melt spinning apparatus illustrated in Fig. 1. A propylene homopolymer having a melt flow rate of 60 g/10 minutes, measured at a load of 2.16 kg and a temperature of 230°C according to ASTM D 1238, was used as a resin used for manufacturing the non-woven fabric. The melting temperature of the resin was set at 200°C, a single-hole discharge rate from a spinning nozzle was set at 0.57 g/min, and the air velocity of cooling air was set as set forth in Table 1. The temperature of upper-stage cooling air and the temperature of lower-stage cooling air were 23°C, the ratio of the height (h₂) of a lower-stage cooling air supply unit (second cooling air supply unit) to the height (h₁) of an upper-stage cooling air supply unit (first cooling air supply unit) was 1, and distance B/distance C was 0.47. The thickness of a partition was one 16th of the height of the upper-stage cooling air supply unit.

A supply unit inlet value set forth in Table 1 refers to the average air velocity value of cooling air supplied to the inlet of the upper-stage cooling air supply unit or the lower-stage cooling air supply unit.

A supply unit outlet value set forth in Table 1 refers to the average air velocity value of cooling air exhausted from the outlet (air-permeable partition) of the upper-stage cooling air supply unit or the lower-stage cooling air supply unit.

An ANEMOMASTER ANEMOMETER (Model 6114) manufactured by KANOMAX was used for measuring an air velocity.

Fig. 2 and Fig. 3 illustrate graphs, each indicating a relationship between the height of a cooling air supply unit and the air velocity (outlet value) of cooling air in Examples 1 to 3 and Comparative Examples 1 to 6. With regard to the height position of the cooling air supply unit, the height position of the upper end of the upper-stage cooling air supply unit corresponds to the upper end of the ordinate of each graph, the height position of the lower end of the lower-stage cooling air supply unit corresponds to the lower end of the ordinate of each graph, and the height position of the partition corresponds to the center of the ordinate of each graph, in Fig. 2 and Fig. 3.

The yarn breakage and yarn fluctuation of non-woven fabrics obtained in Examples 1 to 3 and Comparative Examples 1 to 6 were evaluated for evaluating spinnability.

### <Yarn Breakage>

The yarn breakage was evaluated based on observation results obtained by spinning and forming a melt-kneaded propylene homopolymer consecutively for 10 minutes. The results are set forth in Table 1.

### -Evaluation Criteria-

A: No occurrence of yarn breakage
B: Occurrence of yarn breakage

### <Yarn Fluctuation>

The yarn fluctuation was evaluated by spinning and forming a melt-kneaded propylene homopolymer and observing the state of yarn fluctuation at the position (height position at which the partition was disposed) of the distance B from the nozzle face in the cooling unit. The results are set forth in Table 1.

### -Evaluation Criteria-

A: No occurrence of yarn fluctuation (there is no possibility that the amplitude of the fluctuation of a filament comes into contact with an adjacent filament)
B: Occurrence of yarn fluctuation (there is a possibility that the amplitude of the fluctuation of a filament comes into contact with an adjacent filament)

**[Table 1]**

| | Symbol | Unit | Example 1 | Exampl e 2 | Exampl e 3 | Compar ative Exampl e 1 | Compar ative Exampl e2 | Compar ative Exampl e 3 | Compar ative Exampl e4 | Compar ative Exampl e 5 | Compar ative Exampl e6 |
|---|---|---|---|---|---|---|---|---|---|---|---|
| Distance of Gap | d | mm | 50 | 25 | 10 | 60 | 60 | 0 | 70 | 80 | 100 |
| (Height×Width)/Distance of Gap | (h×L)/d | | 0.061 | 0.123 | 0.307 | 0.051 | 0.051 | - | 0.044 | 0.038 | 0.031 |
| Average Air Velocity of Upper-Stage Cooling Air (Supply Unit Inlet Value) | V₁ | m/s | 0.75 | 0.75 | 0.75 | 0.75 | 0.75 | 0.75 | 0.75 | 0.75 | 0.75 |
| Average Air Velocity of Lower-Stage Cooling Air (Supply Unit Outlet Value) | V₂ | m/s | 1.87 | 1.87 | 1.87 | 1.87 | 1.87 | 1.87 | 1.87 | 1.87 | 1.87 |
| Average Air Velocity Ratio (Supply Unit Inlet Value) | V₁/V₂ | - | 0.40 | 0.40 | 0.40 | 0.40 | 0.40 | 0.40 | 0.40 | 0.40 | 0.40 |
| Average Air Velocity of Upper-Stage Cooling Air (Supply Unit Outlet Value) | V'₁ | m/s | 0.84 | 0.82 | 0.80 | 1.19 | 1.19 | 0.77 | 1.30 | 1.31 | 1.28 |
| Maximum Air Velocity of Upper-Stage Cooling Air (Outlet Value) | V'_{1 max} | m/s | 1.00 | 1.01 | 1.07 | 1.50 | 1.78 | 0.78 | 1.51 | 1.51 | 1.46 |
| Average Air Velocity of Lower-Stage Cooling Air (Supply Unit Outlet Value) | V'₂ | m/s | 1.80 | 1.84 | 1.88 | 1.44 | 1.45 | 1.89 | 1.36 | 1.35 | 1.38 |
| Minimum Air Velocity of Lower-Stage Cooling Air (Outlet Value) | V'_{2 min} | m/s | 1.10 | 1.14 | 1.31 | 0.93 | 0.84 | 1.29 | 0.89 | 0.97 | 1.08 |
| Average Air Velocity Ratio (Supply Unit Outlet Value) | V'₁/V'₂ | - | 0.47 | 0.44 | 0.43 | 0.83 | 0.82 | 0.41 | 0.95 | 0.97 | 0.93 |
| Air Velocity Difference between Upper and Lower Stages | ΔV=V'_{1 max}-V'_{2 min} | m/s | -0.10 | -0.13 | -0.24 | 0.57 | 0.94 | -0.51 | 0.61 | 0.53 | 0.39 |
| Spinnability | Yarn breakage | | A | A | A | B | B | A | B | B | B |
| | Yarn fluctuation | | A | A | A | A | A | B | A | A | A |

As set forth shown in Table 1 and illustrated in Figs. 2 and 3, air velocity difference between upper and lower stages (a value obtained by subtracting the maximum air velocity of a lower stage from the maximum air velocity of an upper stage) in each of Examples 1 to 3 was less than that in each of Comparative Examples 1 to 6, and yarn breakage and yarn fluctuation in Examples 1 to 3 were suppressed.

### Reference Signs List

- 1: Spinning unit
- 2: Nozzle face
- 3: Cooling chamber (cooling unit)
- 4: Cooling air supply unit
- 5: First cooling air supply unit
- 6: Second cooling air supply unit
- 7: Partition
- 8: Air-permeable partition
- 9: Drawing unit
- 10: Filaments
- 100: Melt spinning apparatus

## Claims

1. A melt spinning apparatus (100) comprising:
a spinning unit (1) comprising a plurality of spinning nozzles that spin filaments;
a cooling unit (3) that cools the filaments spun from the spinning nozzles; and
a cooling air supply unit (4) that faces the cooling unit (3) and supplies cooling air to the cooling unit (3) through an air-permeable partition (8),
wherein the cooling air supply unit (4) comprises a first cooling air supply unit (5) at a vertically upper side and a second cooling air supply unit (6) at a vertically lower side, divided into two stages in a vertical direction through a partition (7), there is a gap between an end of the partition (7) facing the air-permeable partition (8) and a face of a side of the air-permeable partition (8) facing the partition (7), and a distance of the gap (d) is 55 mm or less and the distance of the gap (d) is 5 mm or more.

2. The melt spinning apparatus (100) according to claim 1, wherein a ratio of a distance (B) from a nozzle face (2), on which the spinning nozzles of the spinning unit (1) are disposed, to the partition, with respect to the distance of the gap (d), is from 5 to 50.

3. The melt spinning apparatus (100) according to any one of claims 1 to 2, wherein a ratio of a height (h₂) of the second cooling air supply unit, to a height (h₁) of the first cooling air supply unit (5), is from 0.5 to 1.5.

4. The melt spinning apparatus (100) according to any one of claims 1 to 3, wherein a thickness of the air-permeable partition (8) is from 10 mm to 50 mm.

5. The melt spinning apparatus (100) according to any one of claims 1 to 4, wherein a ratio of a thickness of the air-permeable partition (8) to the distance of the gap (d) is from 0.5 to 5.0.

6. The melt spinning apparatus (100) according to any one of claims 1 to 5, wherein the air-permeable partition (8) has a honeycomb shape.

7. The melt spinning apparatus (100) according to any one of claims 1 to 6, wherein the cooling air supply unit comprises a flow regulating plate that regulates the cooling air supplied to the cooling unit, upstream of the air-permeable partition (8), in a direction of cooling air supply.

8. The melt spinning apparatus (100) according to any one of claims 1 to 7, further comprising a first controller that performs control so that a temperature of cooling air supplied to the first cooling air supply unit (5) is from 10°C to 40°C, and a temperature of cooling air supplied to the second cooling air supply unit (6) is higher than the temperature of the cooling air supplied to the first cooling air supply unit (5) by 10°C or more and is from 30°C to 70°C.

9. The melt spinning apparatus (100) according to any one of claims 1 to 8, further comprising a second controller that performs control so that a ratio (V₁/V₂) of an average air velocity (V₁) of cooling air supplied to the first cooling air supply unit (5), with respect to an average air velocity (V₂) of cooling air supplied to the second cooling air supply unit (6), is from more than 0 to 0.7.

10. The melt spinning apparatus (100) according to any one of claims 1 to 9, further comprising a drawing unit that draws the filaments cooled in the cooling unit,
wherein a ratio of a distance (B) from a nozzle face, on which the spinning nozzles of the spinning unit are disposed, to the partition, with respect to a distance (C) from the nozzle face, on which the spinning nozzles of the spinning unit are disposed, to an inlet of the drawing unit, is from 0.2 to 0.8.

11. The melt spinning apparatus (100) according to any one of claims 1 to 10, further comprising a collecting unit that collects cooled and drawn filaments to form a non-woven web, wherein the melt spinning apparatus (100) is used for manufacturing a spunbonded non-woven fabric.

12. A method of manufacturing a non-woven fabric, comprising manufacturing a non-woven fabric from filaments spun from the plurality of spinning nozzles using the melt spinning apparatus (100) according to any one of claims 1 to 11.

13. The method of manufacturing a non-woven fabric according to claim 12, wherein a temperature of cooling air supplied to the first cooling air supply unit (5) is from 10°C to 40°C, and a temperature of cooling air supplied to the second cooling air supply unit (6) is higher than the temperature of the cooling air supplied to the first cooling air supply unit (5) by 10°C or more and is from 30°C to 70°C.

14. The method of manufacturing a non-woven fabric according to claim 12 or 13, wherein a ratio (V₁/V₂) of an average air velocity (V₁) of cooling air supplied to the first cooling air supply unit (5), with respect to an average air velocity (V₂) of cooling air supplied to the second cooling air supply unit (6), is from more than 0 to 0.7.

15. The method of manufacturing a non-woven fabric according to any one of claims 12 to 14, wherein the filaments comprise a propylene-based polymer.

## Patentansprüche

1. Schmelzspinneinrichtung (100), umfassend:
eine Spinneinheit (1), die eine Vielzahl von Spinndüsen umfasst, die Filamente spinnen;
eine Kühleinheit (3), welche die aus den Spinndüsen gesponnenen Filamente kühlt; und
eine Kühlluftzufuhreinheit (4), welche der Kühleinheit (3) gegenüberliegt und der Kühleinheit (3) durch eine luftdurchlässige Trennwand (8) Kühlluft zuführt,
wobei die Kühlluftzufuhreinheit (4) eine erste Kühlluftzufuhreinheit (5) an einer vertikal oberen Seite und eine zweite Kühlluftzufuhreinheit (6) an einer vertikal unteren Seite aufweist, welche in einer vertikalen Richtung durch eine Trennwand (7) in zwei Stufen unterteilt sind, ein Spalt zwischen einem der luftdurchlässigen Trennwand (8) gegenüberliegenden Ende der Trennwand (7) und einer Fläche einer der Trennwand (7) gegenüberliegenden Seite der luftdurchlässigen Trennwand (8) vorhanden ist, und ein Abstand des Spalts (d) 55 mm oder weniger beträgt und der Abstand des Spalts (d) 5 mm oder mehr beträgt.

2. Schmelzspinneinrichtung (100) nach Anspruch 1, wobei ein Verhältnis eines Abstands (B) von einer Düsenfläche (2), auf der die Spinndüsen der Spinneinheit (1) angeordnet sind, zu der Trennwand in Bezug auf den Abstand des Spalts (d) von 5 bis 50 beträgt.

3. Schmelzspinneinrichtung (100) nach einem der Ansprüche 1 bis 2, wobei ein Verhältnis einer Höhe (h₂) der zweiten Kühlluftzufuhreinheit zu einer Höhe (h₁) der ersten Kühlluftzufuhreinheit (5) von 0,5 bis 1,5 beträgt.

4. Schmelzspinneinrichtung (100) nach einem der Ansprüche 1 bis 3, wobei eine Dicke der luftdurchlässigen Trennwand (8) von 10 mm bis 50 mm beträgt.

5. Schmelzspinneinrichtung (100) nach einem der Ansprüche 1 bis 4, wobei ein Verhältnis einer Dicke der luftdurchlässigen Trennwand (8) zu dem Abstand des Spalts (d) von 0,5 bis 5,0 beträgt.

6. Schmelzspinneinrichtung (100) nach einem der Ansprüche 1 bis 5, wobei die luftdurchlässige Trennwand (8) eine Wabenform besitzt.

7. Schmelzspinneinrichtung (100) nach einem der Ansprüche 1 bis 6, wobei die Kühlluftzufuhreinheit eine Flussregulierplatte umfasst, welche die Kühlluft, die der Kühleinheit zugeführt wird, stromaufwärts der luftdurchlässigen Trennwand (8) in einer Kühlluftzufuhrrichtung reguliert.

8. Schmelzspinneinrichtung (100) nach einem der Ansprüche 1 bis 7, weiter umfassend eine erste Steuereinheit, die eine Steuerung derart durchführt, dass eine Temperatur von Kühlluft, die der ersten Kühlluftzufuhreinheit (5) zugeführt wird, von 10°C bis 40°C beträgt und eine Temperatur von Kühlluft, die der zweiten Kühlluftzufuhreinheit (6) zugeführt wird, um 10°C oder mehr höher ist als die Temperatur der Kühlluft, die der ersten Kühlluftzufuhreinheit (5) zugeführt wird, und von 30°C bis 70°C beträgt.

9. Schmelzspinneinrichtung (100) nach einem der Ansprüche 1 bis 8, weiter umfassend eine zweite Steuereinheit, die eine Steuerung derart durchführt, dass ein Verhältnis (V₁/V₂) einer durchschnittlichen Luftgeschwindigkeit (V₁) von Kühlluft, die der ersten Kühlluftzufuhreinheit (5) zugeführt wird, in Bezug auf eine durchschnittliche Luftgeschwindigkeit (V₂) von Kühlluft, die der zweiten Kühlluftzufuhreinheit (6) zugeführt wird, von mehr als 0 bis 0,7 beträgt.

10. Schmelzspinneinrichtung (100) nach einem der Ansprüche 1 bis 9, weiter umfassend eine Zieheinheit, welche die in der Kühleinheit gekühlten Filamente zieht,
wobei ein Verhältnis eines Abstands (B) von einer Düsenfläche, auf der die Spinndüsen der Spinneinheit angeordnet sind, zu der Trennwand in Bezug auf einen Abstand (C) von der Düsenfläche, auf der die Spinndüsen der Spinneinheit angeordnet sind, zu einem Einlass der Zieheinheit von 0,2 bis 0,8 beträgt.

11. Schmelzspinneinrichtung (100) nach einem der Ansprüche 1 bis 10, weiter umfassend eine Sammeleinheit, welche gekühlte und gezogene Filamente sammelt, um eine Vliesbahn zu bilden, wobei die Schmelzspinneinrichtung (100) zum Herstellen eines Spinnvliesstoffs verwendet wird.

12. Verfahren zur Herstellung eines Vliesstoffs, umfassend die Herstellung eines Vliesstoffs aus Filamenten, die aus der Vielzahl von Spinndüsen unter Verwendung der Schmelzspinneinrichtung (100) nach einem der Ansprüche 1 bis 11 gesponnen wurden.

13. Verfahren zur Herstellung eines Vliesstoffs nach Anspruch 12, wobei eine Temperatur von Kühlluft, die der ersten Kühlluftzufuhreinheit (5) zugeführt wird, von 10°C bis
40°C beträgt und eine Temperatur von Kühlluft, die der zweiten Kühlluftzufuhreinheit (6) zugeführt wird, um 10°C oder mehr höher ist als die Temperatur der Kühlluft, die der ersten Kühlluftzufuhreinheit (5) zugeführt wird, und von 30°C bis 70°C beträgt.

14. Verfahren zur Herstellung eines Vliesstoffs nach Anspruch 12 oder 13, wobei ein Verhältnis (V₁/V₂) einer durchschnittlichen Luftgeschwindigkeit (V₁) von Kühlluft, die der ersten Kühlluftzufuhreinheit (5) zugeführt wird, in Bezug auf eine durchschnittliche Luftgeschwindigkeit (V₂) von Kühlluft, die der zweiten Kühlluftzufuhreinheit (6) zugeführt wird, von mehr als 0 bis 0,7 beträgt.

15. Verfahren zur Herstellung eines Vliesstoffs nach einem der Ansprüche 12 bis 14, wobei die Filamente ein Polymer auf Propylenbasis umfassen.

## Revendications

1. Appareil de filage par fusion (100) comprenant :
un poste de filage (1) comprenant une pluralité de buses de filage qui filent des filaments ;
une unité de refroidissement (3) qui refroidit les filaments filés par les buses de filage ; et
une unité d'alimentation en air de refroidissement (4) qui fait face à l'unité de refroidissement (3) et alimente en air de refroidissement (3) l'unité de refroidissement à travers une paroi perméable à l'air (8),
dans lequel l'unité d'alimentation en air de refroidissement (4) comprend une première unité d'alimentation en air de refroidissement (5) au niveau d'un côté verticalement supérieur et une seconde unité d'alimentation en air de refroidissement (6) au niveau d'un côté verticalement inférieur, avec une division en deux niveaux dans la direction verticale par une paroi (7), un espace est présent entre une extrémité de la paroi (7) faisant face à la paroi perméable à l'air (8) et une face d'un côté de la paroi perméable à l'air (8) faisant face à la paroi (7) et une distance sur laquelle s'étend l'espace (d) est égale ou inférieure à 55 mm et la distance sur laquelle s'étend l'espace (d) est égale ou supérieure à 5 mm.

2. Appareil de filage par fusion (100) selon la revendication 1, dans lequel un rapport entre une distance (B) depuis une face à buses (2), sur laquelle les buses de filage du poste de filage (1) sont disposées, et jusqu'à la paroi, et la distance sur laquelle s'étend l'espace (d), varie de 5 à 50.

3. Appareil de filage par fusion (100) selon l'une quelconque des revendications 1 à 2, dans lequel un rapport entre une hauteur (h₂) de la seconde unité d'alimentation en air de refroidissement et une hauteur (h₁) de la première unité d'alimentation en air de refroidissement (5) varie de 0,5 à 1,5.

4. Appareil de filage par fusion (100) selon l'une quelconque des revendications 1 à 3, dans lequel une épaisseur de la paroi perméable à l'air (8) varie de 10 à 50 mm.

5. Appareil de filage par fusion (100) selon l'une quelconque des revendications 1 à 4, dans lequel un rapport entre une épaisseur de la paroi perméable à l'air (8) et la distance sur laquelle s'étend l'espace (d) varie de 0,5 à 5,0.

6. Appareil de filage par fusion (100) selon l'une quelconque des revendications 1 à 5, dans lequel la paroi perméable à l'air (8) présente une forme en nid d'abeille.

7. Appareil de filage par fusion (100) selon l'une quelconque des revendications 1 à 6, dans lequel l'unité d'alimentation en air de refroidissement comprend une plaque de régulation du débit qui régule l'alimentation en air de refroidissement de l'unité de refroidissement, en amont de la paroi perméable à l'air (8), dans une direction d'alimentation en air de refroidissement.

8. Appareil de filage par fusion (100) selon l'une quelconque des revendications 1 à 7, comprenant, en outre, un premier dispositif de commande qui met en œuvre une commande de façon à ce qu'une température de l'air de refroidissement alimentant la première unité d'alimentation en air de refroidissement (5) varie de 10 à 40 °C, et une température de l'air de refroidissement alimentant la seconde unité d'alimentation en air de refroidissement (6) soit supérieure à la température de l'air de refroidissement alimentant la première unité d'alimentation en air de refroidissement (5) d'au moins 10 °C et varie de 30 à 70 °C.

9. Appareil de filage par fusion (100) selon l'une quelconque des revendications 1 à 8, comprenant, en outre, un second dispositif de commande qui met en œuvre une commande de façon à ce qu'un rapport (V₁/V₂) entre une vitesse de l'air moyenne (V₁) de l'air de refroidissement alimentant la première unité d'alimentation en air de refroidissement (5), et une vitesse de l'air moyenne (V₂) de l'air de refroidissement alimentant la seconde unité d'alimentation en air de refroidissement (6) varie de plus de 0 à 0,7.

10. Appareil de filage par fusion (100) selon l'une quelconque des revendications 1 à 9, comprenant, en outre, une unité d'étirage qui étire les filaments refroidis dans l'unité de refroidissement,
dans lequel un rapport entre une distance (B) depuis une face à buses, sur laquelle les buses de filage du poste de filage sont disposées, et jusqu'à la paroi, et une distance (C) depuis la face à buses, sur laquelle les buses de filage du poste de filage sont disposées, et jusqu'à un orifice d'entrée de l'unité d'étirage, varie de 0,2 à 0,8.

11. Appareil de filage par fusion (100) selon l'une quelconque des revendications 1 à 10, comprenant, en outre, une unité de collecte qui collecte les filaments refroidis et étirés pour former une nappe non tissée, dans lequel l'appareil de filage par fusion (100) est utilisé pour fabriquer un non-tissé filé-lié.

12. Procédé de fabrication d'un non-tissé, comprenant la fabrication d'un non-tissé à partir de filaments filés par la pluralité de buses de filage utilisant l'appareil de filage par fusion (100) selon l'une quelconque des revendications 1 à 11.

13. Procédé de fabrication d'un non-tissé selon la revendication 12, dans lequel une température de l'air de refroidissement alimentant la première unité d'alimentation en air de refroidissement (5) varie de 10 à 40 °C, et une température de l'air de refroidissement alimentant la seconde unité d'alimentation en air de refroidissement (6) est supérieure à la température de l'air de refroidissement alimentant la première unité d'alimentation en air de refroidissement (5) d'au moins 10 °C et varie de 30 à 70 °C.

14. Procédé de fabrication d'un non-tissé selon la revendication 12 ou 13, dans lequel un rapport (V₁/V₂) entre une vitesse de l'air moyenne (V₁) de l'air de refroidissement alimentant la première unité d'alimentation en air de refroidissement (5), et une vitesse de l'air moyenne (V₂) de l'air de refroidissement alimentant la seconde unité d'alimentation en air de refroidissement (6), varie de plus de 0 à 0,7.

15. Procédé de fabrication d'un non-tissé selon l'une quelconque des revendications 12 à 14, dans lequel les filaments comprennent un polymère à base de propylène.
